

## UNITED STATES PATENT OFFICE

2,206,711

## METHOD FOR PRODUCING ALLOYS CONTAINING IRON AND CHROMIUM

Marvin J. Udy, Niagara Falls, N. Y.

No Drawing. Application October 16, 1939,  
Serial No. 299,697

11 Claims. (Cl. 75—127)

This invention relates to the production of alloys containing iron and chromium and has for an object the provision of an improved process for producing such alloys. More particularly, the invention contemplates the provision of certain improvements in processes for producing chromium-bearing iron and steel products of low carbon contents.

According to some heretofore customary practices, low-carbon chromium-bearing iron and steel products are formed by adding low-carbon ferrochromium to suitably prepared molten iron or steel baths in suitable furnaces. The low-carbon ferrochromium employed may be produced, for example, by reducing chromite ore with carbon to produce high-carbon ferrochromium, smelting the high-carbon ferrochromium with silica and coke to produce low-carbon, high-silicon ferrochrome silicon and subsequently eliminating the silicon from the ferrochrome silicon by oxidation. Such a procedure for producing low-carbon ferrochromium is expensive. Moreover, the ferrochromium produced is obtained and marketed in the form of a solid relatively high-melting point alloy which can be melted and incorporated in molten iron or steel readily only in furnaces, such as electric furnaces, where large supplies of heat are available.

The addition of solid ferrochromium to molten metal baths causes chilling of the baths. The amount of ferrochromium which can be added efficiently to a molten metal bath in any furnace depends upon the supply of heat available to melt the added ferrochromium and maintain the metal of the bath at the proper temperature. In electric furnaces, ample heat is available for melting commercial ferrochromium and for maintaining alloys of the usual commercial compositions at proper temperatures, so, practically, there is no limit to the amount or proportion of ferrochromium which may be added to molten metal baths in such furnaces. In combustion furnaces such, for example, as open hearth furnaces, on the other hand, the quantities of heat available and the temperatures attainable are limited, and, therefore, only limited quantities of solid ferrochromium may be added effectively to molten metal baths in such furnaces. The chilling effects are limited customarily by employing only high-chromium ferrochromium and thus avoiding the introduction of large quantities of diluent iron, which requires heat for melting, into the molten metal baths with the required amount of chromium. The production of high-

chromium ferrochromium by direct reduction requires the use of high-grade chromite ores which contain suitably high ratios of chromium to iron. Low-grade ores, containing relatively low ratios of chromium to iron require preliminary beneficiation for iron removal prior to reduction for the production of ferrochromium. Because of the necessity for employing high-grade ores or beneficiated ores for the production of ferrochromium according to heretofore customary practices, the production of chromium alloys, such as chromium iron and steel products, is relatively expensive.

It has been proposed also to introduce chromium into low-carbon chromium alloys by reducing chromite ore in contact with molten metal to which the chromium is to be added by means of non-carbonaceous reducing agents. Such proposed procedures have not been highly satisfactory because a large proportion of the chromium is chemically combined in the form of difficultly reducible compounds with magnesia and alumina.

The present invention provides an effective and relatively inexpensive method of producing low-carbon chromium-bearing alloys. According to the invention, chromium is introduced into the furnace in which the alloy is to be made in the form of oxidized ferrochromium. A suitable non-carbonaceous reducing agent capable of reducing to the metallic state the chromium of the oxidized ferrochromium is placed in contact with the oxidized ferrochromium in the furnace. The non-carbonaceous reducing agent, aided by the heat available in the furnace, functions to reduce the iron and chromium of the oxidized ferrochromium, delivering molten metal containing metallic iron and metallic chromium in the proportions in which those elements are present in the oxidized ferrochromium.

The oxidized ferrochromium employed is produced, preferably, by roasting finely divided high-carbon ferrochromium with access of air at an elevated temperature below its fusing temperature and with or without the aid of one or more oxidation promoters. Roasting of the finely divided ferrochromium effects carbon removal by oxidation and also causes oxidation of iron and chromium present in the ferrochromium. The oxidized ferrochromium contains iron and chromium in the proportions in which those elements are present in the ferrochromium subjected to oxidation and in oxidized forms which may be reduced readily by non-carbonaceous reducing agents such, for example, as silicon, ferrosilicon,

ferrochrome silicon and aluminum, and it may be free or largely free of carbon.

Since the process of the invention is capable of delivering molten metal containing iron and chromium in the proportions in which those elements are present in ferro-chromium produced by direct reduction of chromite ore, the invention provides an effective method of adding the chromium of ferrochromium to molten metal baths without chilling the baths. Furthermore, since the process is capable of delivering the metal in the molten state and without chilling molten metal, the necessity for employing high-chromium ferrochromium to avoid the chilling effect of large quantities of iron is eliminated. Thus, it is possible to employ ferrochromium products of any suitable grades, and low-grade ores as well as high-grade ores may be employed in producing such products by direct reduction.

20 The magnesia and alumina of chromite ore are eliminated in the reducing operation which produces the ferrochromium, and the oxidized ferrochromium is free or substantially free of such materials. Consequently, the difficulty of 25 reducing chromium combined with magnesia and alumina encountered in the procedures proposed heretofore for reducing chromite ore in contact with molten metal are not encountered in reducing oxidized ferrochromium in the process of 30 the invention.

Oxidized ferrochromium suitable for use in carrying out the method or process of the invention may be produced, for example, in accordance with any of the procedures outlined in my 35 aforementioned copending application Serial No. 228,860, filed September 7, 1938, which has matured into Patent No. 2,176,688, of which this application is a continuation-in-part.

The ferrochromium may be subjected to the 40 oxidizing treatment alone or in the presence of one or more addition agents such as lime or soda ash which serve as oxidation promoters and which react with the oxides resulting from oxidation of the iron and chromium. When the ferrochromium is subjected to the oxidizing treatment alone in the first instance the product of 45 such oxidizing treatment may be subjected to a further oxidizing treatment in the presence of one or more agents of the aforementioned type to accomplish further oxidation, to bind the oxides chemically, or to accomplish both of these objectives.

Oxidation is readily controlled to form products 50 containing sufficient oxygen to support combustion of reducing agents which may be substantially complete, if desired. The iron of the ferrochromium is converted readily to ferric oxide (Fe<sub>2</sub>O<sub>3</sub>), and the chromium is converted readily to chromic oxide (Cr<sub>2</sub>O<sub>3</sub>). Oxidation may be further controlled to convert a large proportion 55 of the chromium to chromic anhydride (CrO<sub>3</sub>) if desired. Depending upon the conditions under which the oxidized ferrochromium products are to be reduced, they may contain one or more additional oxygen-containing substances such, for example, as sodium nitrate, sodium chlorate and manganese dioxide to provide additional heat for melting the metal and slag produced. When the 60 oxidized ferrochromium is to be reduced in an electric furnace where ample heat is available, it is unnecessary to oxidize the chromium to a state higher than the trivalent state.

Multiple roasting may be carried out with or without the presence of oxidation promoters in 65 any stage, or, when any stage of roasting is car-

ried out in the presence of one or more of such agents, additional amounts may be added to the product of that stage of roasting before subjecting it to the next stage of roasting. Thus, for example, when chromate formation is desired, I 5 prefer to first roast finely divided ferrochromium at a relatively high temperature above 1000° C. in the presence of sufficient lime to form calcium chromite with all of the chromium in the ferrochromium and subsequently roast the product 10 obtained by such roasting treatment at a temperature below 1000° C. in the presence of sufficient additional lime and soda ash to provide a total amount of calcium oxide and sodium oxide 15 to combine with all of the chromic oxide remaining unchanged to form chromate and chromite of calcium and sodium.

Roasting operations may be facilitated by selection of the ferrochromium to be treated. High-carbon ferrochromium products grind more 20 readily and can be converted to desirably small particles more easily than low-carbon ferrochromium. Thus, for example, ferrochromium containing 8 to 10 per cent or more carbon can be reduced to the form of a powder comprising 25 very small particles quite easily; ferrochromium containing 6 to 8 percent carbon is more difficultly reducible to particles of desirably small sizes; and ferrochromium containing less than about 6 percent carbon can be reduced to particles desirably small in size only with considerable 30 difficulty relatively to the difficulties encountered in finely dividing ferrochromium products containing more than 6 percent carbon.

The grinding of relatively low-carbon ferrochromium is facilitated if the ferrochromium also 35 contains silicon. Thus, for example, ferrochromium containing about 4 to 6 percent carbon and amounts of silicon up to about 3 percent can be ground quite readily.

In producing oxidized ferrochromium I prefer 40 to employ ferrochromium as nearly saturated as possible with carbon, or, alternatively, ferrochromium containing smaller amounts of carbon, but containing, also, sufficient silicon to compensate, in its influence upon grinding characteristics, for the carbon deficiency. When I produce 45 the ferrochromium for roasting by reduction treatments of chromium-bearing materials, I prefer to employ sufficient carbon to incorporate in 50 the resulting ferrochromium as much carbon as possible, and, if the conditions of operation are not such as to permit the production of products of the higher carbon content, I operate the reduction process under conditions such as to reduce 55 silicon from silica contained in the charge and form a product containing, preferably, about 1 to 3 percent of silicon. Larger quantities of silicon improve the grinding characteristics of the ferrochromium produced, but they are objectionable 60 because they increase the bulk of the slag produced in the ultimate reduction of the oxidized products of the invention.

I have discovered that oxidation of the iron, 65 chromium and carbon proceeds rapidly and effectively when alloys containing these elements are heated, in a fine state of division, to temperatures substantially higher than 1200° C., but below the melting points of the alloys. At temperatures 70 below 1000° C., oxidation proceeds more slowly, and oxidized products containing less than about 0.30 percent of carbon (by weight) are difficult 75 to obtain. Even at temperatures as high as 1200° C., products containing less than 0.20 percent by weight of carbon are difficult or impossi-

ble to produce with many hours of roasting under oxidizing conditions. At temperatures substantially higher than 1200° C., products containing not more than about 0.10 percent by weight of 5 carbon and containing even as little as a trace of carbon can be produced by roasting under oxidizing conditions for periods of time shorter than two hours. In roasting to effect a high degree of carbon elimination, I prefer to employ temperatures in excess of 1250° C. or even in excess of 10 1300° C. Operating at temperatures above 1300° C., in the range 1300° C. to 1350° C., with and without oxidation promoters, I have obtained 15 oxidized products entirely free of carbon, products in which the presence of carbon could not be detected by the usual analytical methods.

In carrying out roasting of ferrochromium, I 20 may produce oxidized ferrochromium entirely free of carbon or products substantially free of 25 carbon such, for example, as products containing not more than about 0.02 percent or which contain less than about 0.05 percent of carbon. I 30 may produce, also, oxidized products containing carbon in amounts up to 0.10, 0.20, 0.30 percent or 35 more.

According to the preferred method of the invention, the oxidized ferrochromium is added to a molten metal bath in a suitable furnace to form a layer on the surface of the bath in contact with 40 the upper surface of the slag layer if the metal is covered by slag or in contact with the upper surface of the metal if the metal is free or partly free of slag. The non-carbonaceous reducing agent is then placed on top of the layer of oxidized 45 ferrochromium and it functions to reduce the iron and chromium of the oxidized ferrochromium, producing molten metallic iron and molten metallic chromium which enter the molten metal of the bath.

The molten metal bath may be produced and refined or otherwise treated according to customary practices or in any other suitable manner prior to addition of the oxidized ferrochromium. Slag produced in the melting operation may be 50 removed prior to addition of the oxidized ferrochromium, or it may be retained in whole or in part and the oxidized ferrochromium may be added to the upper surface of the slag layer. If the slag produced in the melting operation is removed in whole or in part, a new, clean slag may be provided prior to the addition of the oxidized ferrochromium.

In a preferred method or process of the invention for producing chromium-bearing iron or steel products, I prepare a molten bath of ferrous metal by melting scrap iron or steel or pig iron or other suitable metal products or combinations of metal products in a combustion furnace, electric furnace or other suitable furnace. The melting charge may include suitable slag-forming materials such as lime and silica, and, if desired, the molten bath may be treated with iron oxide to remove carbon from the metal. The slag may then be treated with ferrosilicon to reduce oxides 60 contained therein. All or a portion of the slag may then be removed or the slag may be retained on the surface of the metal. The oxidized ferrochromium may then be placed in the form of a layer on the surface of the molten bath in contact with the slag layer, or in contact with the metal if no slag layer is present, and the reducing agent may be added on top of the layer of oxidized ferrochromium.

The oxidized ferrochromium and the non-carbonaceous reducing agent may be employed in the

form of particles of any suitable sizes. Particles of oxidized ferrochromium about one-half inch (1/2") in size and smaller and particles of non-carbonaceous reducing agent about one-quarter inch (1/4") in size and smaller may be employed 5 satisfactorily. Preferably both the oxidized ferrochromium and the non-carbonaceous reducing agent are employed in the form of particles minus 100-mesh in size.

I prefer to employ silicon-containing materials 10 such as silicon, ferrosilicon, and ferrochrome silicon as the reducing agents. In employing silicon-containing reducing agents, better results are obtained with materials containing more than about fifty (50%) percent of silicon by weight 15 and optimum results are obtained with materials containing not less than about seventy-five (75%) percent of silicon by weight. Materials containing higher percentages of silicon have lower specific gravities and the particles of such 20 materials tend to remain within or on the surface of the layer of oxidized ferrochromium. Silicon contamination of the metal which might result from the use of particles of material of high specific gravities is thus avoided. Gener- 25 ally, it is advisable to determine the particle size of the silicon-containing material to be employed in accordance with the silicon content; in using materials of low silicon content, smaller particles should be used, and in using materials of high 30 silicon content, larger particles may be used.

Lime (CaO) should be provided in sufficient quantity to flux the silica (SiO<sub>2</sub>) or other acid substance formed by oxidation of the reducing agent resulting from reduction of the iron and 35 chromium. Lime may be provided in amount sufficient to produce a calcium silicate slag of any suitable composition, but I prefer to employ lime in an amount sufficient to provide at least one molecule of calcium oxide for each molecule 40 of silica produced. The amount of lime (CaO) added with the oxidized ferrochromium and the reducing agent will depend upon the amount of calcium oxide (CaO) present in the oxidized ferrochromium, that is the lime introduced in carrying out the roasting operation. If an addition of lime is required at the time of adding the oxidized ferrochromium and the reducing agent, I prefer to add the lime in admixture with the reducing agent. In using ferrosilicon, for ex- 45 ample, I may grind the ferrosilicon with the required amount of lime and add the two materials as an intimate mixture to a previously 50 added layer of oxidized ferrochromium.

The reducing agent may be employed in any 55 suitable amount relatively to the amounts of iron and chromium to be reduced from the oxidized ferrochromium. In employing a silicon-containing material, I prefer to employ an amount in excess (up to about ten (10%) percent excess or 60 more) of the amount required theoretically to reduce the iron and chromium of the oxidized ferrochromium. The silicon may be added at one time or at intervals.

The following example illustrates the use of 65 the process of my invention in making high-chromium steel:

In order to make one ton of steel, I melted a charge comprising 1555 pounds of scrap and pig iron in an electric furnace. I then oxidized the 70 carbon with iron oxide, reducing the carbon content to about 0.06 percent. The slag was then highly oxidizing and I added sufficient ferrosilicon containing seventy-five (75%) percent silicon to reduce the iron oxide in the slag and sufficient 75

lime to flux the silica formed in reducing the iron oxide. I then formed a layer of oxidized ferrochromium on the surface of the bath by adding 526 pounds of oxidized ferrochromium analyzing

|                                | Per cent |
|--------------------------------|----------|
| Cr <sub>2</sub> O <sub>3</sub> | 74.0     |
| Fe <sub>2</sub> O <sub>3</sub> | 23.8     |
| CaO                            | 1.47     |
| SiO <sub>2</sub>               | 0.73     |

10 On top of the layer of oxidized ferrochromium, I placed a mixture comprising 217.5 pounds of ferrosilicon containing seventy-five (75%) percent of silicon and 450 pounds of lime in the form 15 of particles one-quarter inch ( $\frac{1}{4}$ ") and smaller in size. The silicon of the ferrochromium reacted with the oxidized iron and chromium of the oxidized ferrochromium, producing molten 20 metallic iron and molten metallic chromium which entered the steel bath. After the reaction was complete, the steel was tapped and finished in the usual manner. The recovery of chromium was about ninety (90%) percent.

I claim:

25 1. The method of producing an alloy containing iron and chromium which comprises forming a molten bath of metallic iron-bearing material in a suitable receptacle, forming a layer of oxidized ferrochromium in finely divided form 30 on the surface of the molten bath, and placing a finely divided silicon-containing reducing agent on the layer of oxidized ferrochromium.

35 2. The method of producing an alloy containing iron and chromium which comprises forming a molten bath of metallic iron-bearing material in a suitable receptacle, forming a layer of oxidized ferrochromium in finely divided form on the surface of the molten bath, and placing a finely divided silicon-containing reducing agent 40 containing not less than about 50 percent of silicon by weight on the layer of oxidized ferrochromium.

45 3. The method of producing an alloy containing iron and chromium which comprises forming a molten bath of metallic iron-bearing material in a suitable receptacle, forming a layer of oxidized ferrochromium in finely divided form on the surface of the molten bath, and placing a finely divided silicon-containing reducing agent 50 containing not less than about 75 percent of silicon by weight on the layer of oxidized ferrochromium.

55 4. The method of producing chromium-bearing steel which comprises heating a charge comprising steel scrap and slag-forming materials and forming a slag-covered molten metal bath, treating the molten bath with iron oxide to remove carbon from the metal, treating the resulting slag with a reducing agent to remove excess iron oxide, subsequently forming a layer of oxidized ferrochromium on the surface of the molten bath, and placing a finely divided silicon-containing reducing agent on the layer of oxidized ferrochromium.

60 5. The method of producing an alloy contain-

ing iron and chromium which comprises forming a molten bath of metallic iron-bearing material in a suitable receptacle, forming a layer of oxidized ferrochromium in finely divided form on the surface of the molten bath, and placing finely divided ferrosilicon on the layer of oxidized ferrochromium. 5

6. The method of producing an alloy containing iron and chromium which comprises forming a molten bath of metallic iron-bearing material 10 in a suitable receptacle, forming a layer of oxidized ferrochromium in finely divided form on the surface of the molten bath, and placing finely divided ferrochrome silicon on the layer of oxidized ferrochromium. 15

7. The method of producing an alloy containing iron and chromium which comprises forming a molten bath of metallic iron-bearing material in a suitable receptacle, forming a layer of oxidized ferrochromium in solid, finely divided form 20 on the surface of the molten bath, and placing lime and a silicon-containing reducing agent on the layer of oxidized ferrochromium.

8. The method of producing an alloy containing iron and chromium which comprises forming a molten bath of metallic iron-bearing material 25 in a suitable receptacle, forming a layer of oxidized ferrochromium in solid, finely divided form on the surface of the bath, and placing an intimate mixture of lime and a silicon-containing 30 reducing agent on the layer of oxidized ferrochromium.

9. The method of producing an alloy containing iron and chromium which comprises forming a molten bath of metallic iron-bearing material 35 in a suitable receptacle, forming a layer of oxidized ferrochromium in finely divided form on the surface of the molten bath, and placing a finely divided non-carbonaceous reducing agent on the layer of oxidized ferrochromium. 40

10. The method of producing an alloy containing iron and chromium which comprises forming a molten bath of metallic iron-bearing material in a suitable receptacle, forming a layer of oxidized ferrochromium in finely divided form on 45 the surface of the molten bath, and placing a finely divided silicon-containing reducing agent on the layer of oxidized ferrochromium, the major portions of said oxidized ferrochromium and said reducing agent consisting of particles minus 100- 50 mesh in size.

11. The method of producing an alloy containing iron and chromium which comprises forming a molten bath of metallic iron-bearing material in a suitable receptacle, forming a layer of oxidized ferrochromium in finely divided form on the surface of the molten bath, and placing a finely divided silicon-containing reducing agent on the layer of oxidized ferrochromium, the major portion of said oxidized ferrochromium 55 consisting of particles smaller than one-half inch in size and the major portion of said reducing agent consisting of particles smaller than one-quarter inch in size.